

Sept. 1, 1953

H. F. SHANNON

2,650,889

**H. F. SHANNON**  
METHOD AND APPARATUS FOR INHIBITING ROLL PICKUP  
IN CONTINUOUS ANNEALING OF STEEL STRIP  
Filed May 18, 1950

Filed May 18, 1950

FIG. 1.



FIG. 3.



FIG. 2.



FIG. 4.



*Inventor:*

HARRY F. SHANNON,  
By: Donald G. Adcock  
his Attorney.

## UNITED STATES PATENT OFFICE

2,650,889

METHOD AND APPARATUS FOR INHIBITING  
ROLL PICKUP IN CONTINUOUS ANNEAL-  
ING OF STEEL STRIPHarry F. Shannon, Pittsburgh, Pa., assignor to  
United States Steel Corporation, a corporation  
of New Jersey

Application May 18, 1950, Serial No. 162,669

6 Claims. (Cl. 148—21.5)

1

This invention relates to provisions for inhibiting "roll pick-up" in the continuous heat-treatment of flat-rolled metal products.

The processing of certain classes of flat-rolled metal products, e. g., steel strip, and particularly silicon-steel strip from which electrical sheets are sheared, preferably includes annealing or normalizing, usually in a decarburizing atmosphere. This treatment is customarily effected by the use of a continuous furnace having driven rolls for supporting the product and conveying it therethrough. The rolls which may be of ordinary steel or a heat-resistant alloy, show a strong tendency to pick up particles of combined silicon and iron oxide within a relatively short time. The oxides of iron and silicon, separately, have high melting points but when combined in the proper amounts they form the compound known as fayalite which has a relatively low melting point. This compound forms on the surfaces of silicon-steel strip during continuous annealing at elevated temperatures in an oxidizing atmosphere. Particles of the fayalite thus formed are tacky at the operating temperature of the furnace and adhere to the surface of the metal conveyor rolls, thereby forming so-called pick-up spots. The particles build up in localized areas forming projections on the rolls which mark the strip in a manner designated as "dimpling." This renders the material unusable for most purposes. As a result, it frequently becomes necessary to shut down the furnace and clean off the rolls with the attendant increase in maintenance cost and loss of production.

I have invented a novel method for inhibiting oxide pick-up by the rolls of a continuous furnace and apparatus for carrying out such method easily, conveniently and effectively. My method contemplates the maintenance on the conveyor rolls of a film of a material which is not wet by the iron and silicon oxides on the strip, thus preventing their adherence to the metal of the rolls. The material used to form a film on the surface of the rolls may be graphite or other refractory material such as metallic oxides. The apparatus of my invention includes means for supporting a mass of the film-forming material in contact with the rolls traversed by the product, so as to have wiping engagement with the roll surfaces.

A complete understanding of the invention may be obtained from the following detailed description and explanation thereof which refer to the accompanying drawings illustrating a pre-

2

ferred embodiment and a modification. In the drawings,

Figure 1 is a central vertical section, largely diagrammatic, taken longitudinally through a continuous strip-annealing furnace having the invention incorporated therein;

Figure 2 is a partial horizontal section taken along the plane of line II—II of Figure 1, showing parts in plan;

Figure 3 is a view partly in elevation and partly in section, taken along the plane of line III—III of Figure 1; and

Figure 4 is a transverse section through one of the conveyor rolls taken along the plane of line IV—IV of Figure 3.

Referring in detail to the drawings and, for the present, to Figure 1, a strip-annealing furnace indicated generally at 10 comprises a refractory-lined enclosure laid up within a conventional binding fabricated from steel plate and rolled sections (not shown) in the known manner. The furnace has an entrance opening 11 at one end and an exit opening 12 at the other adapted to permit the passage of strip therethrough from an uncoiler at the entrance end to a recoiler at the exit end. The furnace may be heated by any suitable means, i. e., electric resistors, radiant combustion tubes or the like. A controlled atmosphere, usually decarburizing, is supplied to the furnace chamber by any convenient means (not shown).

In order to maintain each point along the strip at the temperature necessary to produce decarburization, for the required length of time, the strip is trained alternately over conveyor rolls 13 in an upper series designated 13<sup>a</sup> and a lower series designated 13<sup>b</sup>. The rolls 13 have shafts 14 extending through the side walls of the furnace and journaled in any suitable bearings carried thereby. The shafts are driven in the known manner by any convenient mechanism. The arrangement of the rolls in the two series as shown is such that the strip, when properly trained thereover is caused to make a plurality of passes upwardly and downwardly throughout substantially the full height of the chamber. The cylindrical bodies of the rolls may be fabricated from steel plate. Instead of a unitary cylinder, the roll bodies may consist of a plurality of discs spaced along the shaft.

Baffles 15 and 16 divide the interior of the furnace chamber into several chutes traversed successively by the strip in its alternate upward and downward passes. A cradle 17 of steel bars, pref-

erably heat-resistant steel, is positioned above each lower roll 13<sup>a</sup>, the ends of the bars being embedded in the baffles and furnace walls. A block of graphite 18 is loosely confined in each cradle and rides on the roll therebelow. On rotation of the roll, it wipes the block and thereby acquires a film of graphite on its surface. This film is not wet by the oxides on the surface of the strip traveling around the roll and the latter therefore does not pick up such oxides. As a result, the roll surface remains clean and smooth over a long period of operation and the strip is consequently not marked by its contact therewith. Short pieces of bar 17<sup>a</sup> welded to the cradle prevent tilting of the blocks 18.

The upper rolls 13<sup>a</sup> have tables 19 therebelow on which graphite blocks 18 are loosely confined as by an edge flange or the like. Each table is carried on a tilting frame 20 pivoted at 21 to the side walls of the furnace. A counterweight 22 suspended from the outer end of each frame constantly urges the blocks 18 on tables 19 into wiping engagement with rolls 13<sup>a</sup> for the purpose of applying a graphite film thereto. The table and frame are preferably of heat-resistant steel.

Instead of graphite, I may utilize as the film-forming material refractory metal oxides such as magnesia, alumina and silica. The silica may be in the form of diatomaceous earth. These oxides may, like the graphite, be molded to appropriate shape by the use of a suitable binder, to give them the block form illustrated. Another material which may be used is molybdenum disulphide. It is generally similar to graphite in its effect for the purpose of this invention.

Experience shows that the invention permits the operation of a continuous strip-annealing furnace for much longer periods than otherwise possible, without the occurrence of roll pick-up to an objectionable degree. The invention thus materially reduces the maintenance cost of the furnace and increases its production.

I claim:

1. In a method of treating silicon-steel strip, 45

the steps including passing the strip in single ply through a continuous furnace, supporting the strip in the furnace on metal rolls and continuously applying to said rolls a film of refractory material thereto thereby inhibiting the adherence thereto of oxides formed on the strip.

2. The method defined by claim 1 characterized by said material being graphite.

3. The method defined by claim 1 characterized by said material being selected from the group consisting of magnesia, alumina and silica.

4. The combination with a strip-annealing furnace having horizontal metal conveyor rolls extending thereacross, of a pair of bars mounted on the interior of the furnace walls adjacent each roll and a mass of refractory material carried by said bars in contact with said roll, continuously applying thereto a film inhibiting the picking up of oxides from the strip.

5. The combination defined by claim 4 characterized by said bars forming a cradle above the roll adapted to confine said mass.

6. The combination defined by claim 4 characterized by a table below the roll supported on said bars and counterbalancing means urging the table upwardly toward the roll, said means being carried on said bars.

HARRY F. SHANNON.

References Cited in the file of this patent

UNITED STATES PATENTS

| Number    | Name               | Date           |
|-----------|--------------------|----------------|
| 669,765   | Reichhelm          | Mar. 12, 1901  |
| 1,626,685 | Marden et al.      | May 3, 1927    |
| 1,765,955 | Von Maltitz et al. | June 24, 1930  |
| 1,956,401 | Russ               | Apr. 24, 1934  |
| 2,057,518 | Fraser et al.      | Oct. 13, 1936  |
| 2,058,447 | Hazelett           | Oct. 27, 1936  |
| 2,183,010 | Coxe               | Dec. 12, 1939  |
| 2,199,191 | Tour               | Apr. 30, 1940  |
| 2,345,181 | Cooper et al.      | Mar. 28, 1944  |
| 2,428,344 | Stookey            | Sept. 30, 1947 |
| 2,534,973 | Ipsen et al.       | Dec. 19, 1950  |
| 2,603,578 | Ornitz             | July 15, 1952  |